# EUROPEAN PATENT SPECIFICATION

(11) **EP 0 073 615 B1**
(45) Date of publication and mention of the grant of the patent: **04.06.1986**
(21) Application number: 82304401.1
(22) Date of filing: 20.08.1982
(51) Int. Cl.: C10L 1/18, C10L 1/24

(54) **Residual fuel oil compositions and the preparation and combustion thereof**
Zusammensetzung aus Heizölrückständen, deren Herstellung und Verbrennung
Des compositions d'huile combustible résiduelle et la préparation et la combustion de ceux-ci

(30) Priority: 25.08.1981 US 296016
(43) Date of publication of application: 09.03.1983
(73) Proprietor: EXXON RESEARCH AND ENGINEERING COMPANY, Florham Park, New Jersey 07932-0390 (US)
(72) Inventor: Feldman, Nicholas, Woodbridge New Jersey (US)
(74) Representative: Pitkin, Robert Wilfred

## Description

This invention relates to residual fuel oil compositions and the preparation and combustion thereof, which fuel oil compositions contain certain zirconium salts to reduce the amount of particulate matter formed during combustion.

Residual fuel oils, including Grades Nos. 4, 5 and 6 (ASTM D-396), are widely used in a variety of industrial heating and steam boiler applications. A particularly desired fuel oil is No. 6, which is extensively used by utility and power companies.

State, federal, EPA, and other, emission standards currently limit the use of residual fuels which produce excessive amounts of particulate emission during combustion and thus are not in compliance with standards.

However, the situation is relatively complicated, since country-to-country, or state- to-state, emission standards tend to be different and compliance by a residual fuel oil in one location may not necessarily be achieved in another. Further, since standards are continuously subject to change, a residual fuel oil currently in compliance with emission standards may not be in compliance in the near future in the same location and under the same end-use conditions.

Residual fuel oils which tend to produce excessive amounts of particulate emission generally have one or more characteristics associated with them: a sulfur content above about 1 percent; a Conradson Carbon Residue (ASTM D-189, also termed "Con Carbon" in the art) above about 7 percent; or a high asphaltene content. Residual fuel oils yielding particulate emissions that surpass the existing standards can't be directly used, but in some cases can be blended in admixture with fuels that do meet existing standards, which are generally low in sulfur and/or low in "Con Carbon" and asphaltene content. This situation has resulted in an overall increased demand for fuel oils which meet emission standards despite their diminishing supply and attendant increase in cost.

What is desired is a process for increasing the utility of these high emission yielding residual fuels oils for industrial heating purposes in a manner that results in acceptable particulate emissions, despite a high sulfur content, a high Con Carbon residue and/or high asphaltene content.

In the area of related problems, it is known in the art that the use of specific additives in certain hydrocarbon fuels, can reduce smoke or soot upon combustion, in certain instances. It is also known to use specifc additives in fuels to inhibit corrosion, inhibit slag formation in boilers and to reduce the deleterious effect of vanadium present, in such fuels.

GB-A-837407 discloses improving the combustion characteristics of a fuel oil composition, particularly a diesel engine fuel oil, by adding a small proportion of sulfonates of at least two metals of Group IV of the Periodic Table. The superiority of employing the sulphonates of both tin and lead over either used alone is illustrated.

DE-A-2316230 discloses residual fuel oils, particularly marine diesel fuel oils, containing (a) a fuel oil soluble compound of magnesium, aluminium, silicon, calcium, strontium or barium or mixtures thereof; (b) a fuel oil soluble compound of zirconium or titanium, the components (a) and (b) being present in an amount to provide a weight ratio of aluminium, silicon, calcium, barium or mixtures thereof to zirconium or titanium of from 2:1 to 15:1. The use of such a two-component additive is said to be for the purpose of minimizing the deleterious effects associated with the combustion of a vanadium containing residual fuel oil by producing fluffy, friable, high melting deposits of a less adhesive and less corrosive nature.

In accordance with this invention, there is provided a residual fuel oil composition, characterised by a residual fuel oil composition, characterised by a residual fuel, preferably a No. 6, fuel oil, having present therein an amount of an additive consisting essentially of at least one zirconium salt selected from oil-soluble zirconium salts of (i) alcohols or phenols having the formula ROH, where R is a hydrocarbyl group of 2 to 24 carbon atoms, or (ii) sulfonic acids having the formula RS0₃H, where R is an alkyl, cycloalkyl, aryl, alkaryl or aralkyl group, the sulfonate salt having molecular weight of up to 2500; said amount of the additive being from 1 to 1000 parts per million, by weight, calculated as metallic zirconium.

Further, according to the invention there is provided a process of preparing a residual fuel oil, preferably a No. 6 fuel oil, characterised by dissolving in said fuel oil an amount of an additive consisting essentially of at least one zirconium salt selected from oil-soluble zirconium salts of (i) alcohols or phenols having the formula ROH, where R is a hydrocarbyl group of 2 to 24 carbon atoms, or (ii) sulfonic acids having the formula RS0₃H, where R is an alkyl, cycloalkyl, aryl, alkaryl or aralkyl group, the sulfonate salt having a molecular weight of up to 2500; said amount of the additive employed being 1 to 1000 parts per million preferably 50 to 150 parts per million, by weight, calculated as metallic zirconium.

It has unexpectedly been found that by adding a selected said oil-soluble zirconium salts of an alcohol/phenol or sulfonate to a residual fuel oil, and particularly No. 6 fuel oil, the amount of particulate matter formed during combustion can be significantly reduced in amounts of 10 to 25 percent or greater.

The term "residual fuel oil" as used herein, is well-known and as described hereinabove, and includes Grades No. 4, No. 5 and No. 6 residual fuels oils, meeting the specifications of ASTM D-396. Particularly preferred is No. 6 fuel oil.

The reason these particular zirconium additives exhibit this surprising effect is not clearly understood. It may be that the subject compounds promote and activate the complete oxidation of hydrocarbon and sulfur-containing constituents in the fuel to volatile or gasesous compounds during combustion, in a highly specific manner. The subject zirconium salts or compounds, also termed "additives" herein operative in the instant invention, comprise oil soluble zirconium salts of an alcohol/phenol or sulfonate. The zirconium salt of selected alcohols or phenols will be a zirconium salt of an alcohol or phenol having the formula: where R is a hydrocarbyl group of 2 to 24 carbon atoms. More particularly R is a branched or unbranched, hydrocarbyl group preferably having 2 to 13 carbon atoms. Preferred compounds are those where R is a saturated or unsaturated aliphatic group having 2 to 8 and more preferably 3 to 4 carbons. Most preferred are those compounds where R is a saturated aliphatic group, and particularly those having 3 to 4 carbons. Compounds of this type include R groups which may be alkyl, aryl, alkaryl, aralkyl and alkenyl. Illustrative alcohol or phenol compounds of this type include ethanol, propanol, butanol, hexanol, decanol, octadecanol, eicosanol, phenol, benzyl alcohol, xylenol, naphthol, ethyl phenol, crotyl alcohol etc. Further information and description of the useful alcohols of this type may be found in Kirk-Othmer, "Encylopedia of Chemical Technology" Second Edition, 1963 Vol. 1, pp 531-638.

The zirconium salt of sulfonic acids useful in this invention are the zirconium salts of sulfonic acids having the formula: where R is a hydrocarbyl group having 2 to 200 and preferably 10 to 60 carbon atoms. More particularly, the R group in said sulfonic acids will be an alkyl, cycloalkyl, aryl, alkaryl or aralkyl and said salt will have a molecular weight of about 100 to about 2500, preferably about 200 to about 700.

The sulfonic acids are characterized by the presence of the sulfo group -S0₃H (or -S0₂0H) and can be considered derivatives of sulfuric acid with one of the hydroxyl groups replaced by an organic radical. Compounds of this type are generally obtained by the treatment of petroleum fractions (petroleum sulfonates). Because of the varying natures of crude oils and the particular oil fraction used, sulfonates generally constitute a complex mixture and it is best to define them in a general manner giving the molecular weight as defined above. Particularly preferred sulfonates are those having an alkaryl group, i.e. alkylated benzene or alkylated naphtalene.

Illustrative examples of sulfonic acids useful in this invention are: dioctyl benzene sulfonic acid, dodecyl benzene sulfonic acid, didodecyl benzene sulfonic acid, dinonyl naphthalene sulfonic acid, dilauryl benzene sulfonic acid, lauryl cetyl benzene sulfonic acid, polyolefin alkylated benzene sulfonic acid such as polybutylene and polypropylene, etc. Further details regarding sulfonic acids may be found in Kirk-Othmer, "Encyclopedia of Chemical Technology", Second Edition, 1969, Vol. 19 pp 311 to 319 and in "Petroleum Sulphonates" by R. Leslie in Manufacturing Chemist, October 1950 (XX1, 10) pp 417 to 422.

Methods of preparing the subject zirconium salts described above are well known in the art and generally said salts are commercially available.

The zirconium additive is incorporated into the residual fuel oil by dissolving therein. This is accomplished by conventional methods, for example heating, stirring.

The amount of zirconium additive to be used is 1 to 1000 ppm by weight and preferably 10-500 ppm by weight in said fuel oil, and particularly preferred 50 to 150 ppm by weight zirconium additive, taken as metallic zirconium; the abbreviation "ppm" meaning "parts per million".

By the term "reduce the amount of particulate matter formed during combustion", as used herein, is meant that normally at least about a five percent reduction in formed particulate matter, and preferably from about 10 to 25 percent and greater, reduction in formed particulate matter is achieved as compared to the combustion of the residual fuel oil in the absence of the subject zirconium additive.

In the process, the fuel oil containing said additive is generally mixed with oxygen, usually in the form of air, to form a fuel/air mixture prior to combustion. Generally, the amount of air utilized is an excess over the stoichiometric amount to completely combust the fuel oil to carbon dioxide and water. The reason for utilizing this excess is that complete mixing does not always occur between the fuel oil and the air, and that also a slight excess of air is desirable since it serves to reduce the tendency of soot and smoke formation during combustion. Generally, the excess of air used is about 2 to 35 percent (0.4 to 7 percent based on oxygen) over the stoichiometric amount depending upon the actual end-use conditions which may vary considerably from one type of industrial boiler to the next. One disadvantage in using a large excess of air is that a greater amount of heat is lost through entrainment that would otherwise be utilized for direct heating purposes. We have found that by use of the subject zirconium additives, less excess air is required to reduce smoke and soot formation and thus the heating efficiency of the residual fuel oil is greater, as well as resulting in a reduction of particulate emission.

The above-described step of mixing fuel oil and air is conventional and is usually accomplished for example, by steam or air atomization to produce a fine spray which is then combusted to maintain and support a flame. The combustion is controlled and conducted at a particular "firing rate" which is usually expressed as Ibs/minute of fuel oil combusted.

The combustion of residual fuel oil is usually carried out in conventional industrial boilers, utility boilers, refinery furnaces and the like. The amount of particulate matter formed during combustion of residual fuel oil will vary over a broad range and is dependent upon a number of factors such as type of boiler, boiler size, number and type of burners, source of the residual fuel oil used, amount of excess air or oxygen, firing rate and the like. Generally, the amount of particulate matter formed will be in the range of about 0.01 to 1.0 weight percent of the fuel oil used and higher. One weight percent corresponds to one gram particulate matter formed from the combustion of 100 grams of fuel oil. The amount of particulate matter formed, herein termed "total particulate matter," is actually the sum of two separate measurements; "tube-deposits", the amount of particulate matter deposited inside of the boiler, and two, "filtered stack particulate", which is the amount of particulate matter formed which escapes the boiler and is actually emitted out of the stack into the air. EPA measurements are generally only concerned with filtered stack particulate which is directly released into the air environment and contributes to a decrease in air quality. However, "tube deposits" lead to corrosion of the equipment, frequent "clean-outs" and add to the total operating costs. Furthermore, as tube deposits collect on the inside of the apparatus, a critical crust thickness is reached and further tube deposits are then entrained in stack particulate, which significantly increases the amount of particulate emission. Thus, in order to fully assess the overall operating advantages of a particular residual fuel oil in a boiler operation, the amount of tube deposits should also be considered, as well as total stack particulate for compliance with emission standards.

The amount of allowed stack particulate will vary from state to state and is also subject to a minimum amount allowed under Federal EPA standards. For example, in Florida, the currently allowable limit for existing power plants is 45.4 g (0.10 lbs) particulate emission 1.06 MJ (per million BTU), which is equivalent to about 0.185 weight percent of particulate stack emission per weight of combusted fuel oil. Since the allowable emission standards will vary from jurisdiction to jurisdiction, differing amounts of the subject zirconium additive will be necessary to produce a residual fuel oil composition in compliance with those standards.

Measurement of the amount of "stack particulate matter" is conducted by EPA Method #5 Stack Sampling System, "Determination of Particulate Emissions from Stationary Sources" and is described in the Federal Register.

The particulate stack emissions are generally comprised of particulate carbon, sulfur-containing hydrocarbons, inorganic sulfates and the like.

The following examples are illustrative of this invention and should not be construed as being limitations on the scope and spirit of such invention.

### Example 1

Combustion runs were carried out in a 37.3 kW (50 horsepower) ABCO, 2-pass, water jacketed forced draft boiler with an air-atomizing burner and a nominal firing rate of 0.54 Kg/min (1.2 lbs/min) of residual fuel oil. The boiler was modified so that closure on each end could be opened easily for recovery of deposits laid down in the boiler. Two other modifications included installation of a second fuel system so the boiler could be heated to operating temperatures on No. 2 oil and then switched over to the test fuel without shutting down or upsetting the boiler operation unduly and installation of a two foot length of firebrick lining at the burner end of the firetube and a Cleaver-Brooks nozzle assembly in place of the Monarch nozzle. These modifications eliminated oil pooling and rapid carbon deposits on the firetube walls when residual fuel was fired. The first pass is a 49 cm (18.375 in.) diameterx178 cm (5 ft. 10 in.) long fire tube; the second pass consists of 52 tubes each 6 cm (2.375 in.) diameterx188 cm (6 ft. 2 in.) long.

Atomization of the fuel was accomplished using a low pressure air-atomizing nozzle. Viscosity of the fuel oil at the nozzle was maintained at 30 centistokes by heating the oil to a predetermined temperature (about 105°C). Prior to contacting the burner gun, the atomized fuel oil was mixed with a measured amount of excess "secondary" air which was forced through a diffuser plate to insure efficient combustion. The secondary air was provided by a centrifugal blower mounted in the boiler head. The amount of secondary air was controlled by means of a damper which was regulated to keep the oxygen level in the atomized fuel at about 1.5% in excess (over that needed stoichiometrically to completely combust the fuel).

A run was started by firing the boiler and heating itto operating temperature for 55 minutes using No. 2 oil. The feed was then switched to test fuel and after allowing sufficient time for conditions to stabilize (about 25 minutes) samples of about 10 minutes duration were collected isokinetically from the stack on tared, Gelman, Type A (20.3x25.4 cm) fiber glass filters. The test fuel was a No. 6 fuel oil.

Total particulate matter formed was determined by adding the amount of Stack particulate measured isokinetically (EPA Method 5 Stack Sampling System) to the amount deposited in the tubes of the boiler i.e. "tube deposits".

The EPA Method 5 Stack Sampling System was conducted with a commercially available system for this purpose. This unit consisted of an 0.46 m (18-inch) glass lined probe, a cyclone, a 125 mm glass fiber filter and four impingers. The first two impingers contained water, the third was empty and the last one contained silica gel. With the exception of the impingers, the entire sampling train was maintained at about 175°C to insure that the stack gases entering the sampling system were above the H_{I}S0₄ dew point.

The deposits laid down in each of the 52 tubes is collected on a separate, tared 20.3x25.4 cm fibre-glass filter. Deposits are collected by positioning a specially-designed filter holder against the end of each tube in turn, pulling air through the tube and the filter using a high-volume vacuum pump and manually brushing the tube from end-to-end ten times with 0.064 m (2.50 inch) diameter wire shank brush. The brush is mounted on a 2.44 m (8 ft) long, 0.006 m (0.25 in.) diam. SS rod driven by an electric drill. This method gives almost 100% recovery of the deposits laid down in the tubes. All the tubes are sampled because for a given run there are large differences in deposit weight from tube-to-tube in each row of tubes across the boiler and from top row to bottom row and there is no consistent ratio of the weight of deposit collected from a given tube from run-to-run.

The fuel oil used (Test Fuel) in the runs analyzed for the following constituents:

The zirconium additive used in the run was zirconium propoxide an alcohol salt and was present in a concentration of 100 ppm taken as metallic zirconium.

For test fuel alone, the stack particulate was 0.34 wt% on fuel, while the tube deposits was 0.20 wt% on fuel for a total test particulate wt% of 0.54. The sample of fuel containing the zirconium propoxide measured a stack particulate of 0.24 wt% on fuel and tube deposits of 0.16 wt% on fuel for a total particulate wt% of 0.40. The improvement in using the zirconium additives was a reduction in total particulates of 25.9%.

### Example 2

Following the same general procedure and using the ABCO boiler described in Example 1, a sample run using 100 ppm of a zirconium sulfonate additive, i.e. zirconium salt of dodecyl benzene sulfonic acid, was made with the same No. 6 fuel oil as in said Example 1.

The results of the sample containing zirconium sulfonate were a stack particulate of 0.29 wt% on fuel and tube deposits of 0.18 wt% on fuel for a total particulate of 0.47 wt% on fuel. The improvement in using the zirconium additive was a reduction in total particulate of 13.0%.

## Claims

1. A residual fuel oil composition, characterised by a residual fuel, preferably a No. 6 fuel oil, having present therein an amount of an additive consisting essentially of at least one zirconium salt selected from oil-soluble zirconium salts of (i) alcohols or phenols having the formula ROH, where R is a hydrocarbyl group of 2 to 24 carbon atoms, or (ii) sulfonic acids having the formula RS0₃H, where R is an alkyl, cycloalkyl, aryl, alkaryl or aralkyl group, the sulfonate salt having a molecular weight of up to 2500; said amount of the additive being from 1 to 1000 parts per million, by weight, calculated as metallic zirconium.

2. A residual fuel oil composition as claimed in claim 1, characterised in that the zirconium salt of salts is or are present in a total amount of from 50 to 150 ppm, by weight, calculated as metallic zirconium.

3. A composition as claimed in claim 1 or claim 2, wherein the R group is said alcohol salt is a saturated or unsaturated aliphatic group having 2 to 8 carbons.

4. A composition as claimed in claim 1 or claim 2, wherein the R group in said sulfonic acid is an alkaryl group and the salt has a molecular weight of 200 to 700.

5. A residual fuel oil composition as claimed in claim 1 or claim 2, characterised in that the zirconium salt or salts is or are selected from zirconium propoxide, zirconium dodecyl benzene sulfonate, or mixtures thereof.

6. A process of preparing a residual fuel oil, preferably a No. 6 fuel oil, characterised by dissolving in said fuel oil an amount of an additive consisting essentially of at least one zirconium salt selected from oil-soluble zirconium salts of (i) alcohols or phenols having the formula ROH, where R is a hydrocarbyl group of 2 to 24 carbon atoms, or (ii) sulfonic acids having the formula RS0₃H, where R is an alkyl, cycloalkyl, aryl, alkaryl or aralkyl group, the sulfonate salt having a molecular weight of up to 2500; said amount of the additive employed being 1 to 1000 parts per million, preferably 50 to 150 parts per million, by weight, calculated as metallic zirconium.

7. A composition as claimed in claim 6, wherein said fuel oil contains above 1 weight percent sulfur.

8. A process in which a residual fuel oil, preferably a No. 6 fuel oil is combusted; characterised by
(a) dissolving in the fuel oil an amount defined in claim 1 or claim 2 of at least one zirconium salt defined in any one of claims 1 and 3 to 5, and
(b) combusting the resultant residual fuel oil composition.

## Patentansprüche

1. Rückstandsheizölzusammensetzung, gekennzeichnet durch einen Rückstandsheizöl, vorzugsweise ein Nummer 6 Heizöl, das einen Gehalt eines Additivs aufweist welches im wesentlichen aus mindestens einem Zirkoniumsalz auggewählt aus öllöslichen Zirkoniumsalzen von (i) Alkoholen oder Phenolen mit der Formel ROH, in der R eine Hydrocarbylgruppe mit 2 bis 24 Kohlenstoffatomen ist, oder (ii) Sulfonsäuren mit der Formel RS0₃H besteht, worin R eine Alkyl-, Cycloalkyl-Aryl-, Alkaryl- oder Aralkylgruppe ist, wobei das Sulfonatsalz ein Molekulargewicht von bis zu 2500 besitzt und die Menge des Additivs berechnet als metallisches Zirkonium 1 bis 1000 Gew. ppm beträgt.

2. Rückstandsheizölzusammensetzung nach Anspruch 1, dadurch gekennzeichnet, daß das Zirkoniumsalz oder die Zirkoniumsalze berechnet als metallisches Zirkonium in einer Gesamtmenge von 50 bis 150 Gew. ppm vorhanden sind.

3. Zusammensetzung nach Anspruch 1 oder 2, dadurch gekennzeichnet, daß die R-Gruppe im Alkoholsalz eine gesättigte oder ungesättigte aliphatische Gruppe mit 2 bis 8 Kohlenstoffatomen ist.

4. Zusammensetzung nach Anspruch 1 oder 2, dadurch gekennzeichnet, daß die R-Gruppe in der Sulfonsäure eine Alkyrylgruppe ist und das Salz ein Moleulargewicht von 200 bis 700 besitzt.

5. Rückstandsheizölzusammensetzung nach Anspruch 1 oder 2, dadurch gekennzeichnet, daß der Zirkoniumsalz oder die Zirkoniumsalze ausgewählt sind aus Zirkoniumpropoxid, Zirkoniumdodecylbenzosulfonat oder Mischungen derselben.

6. Verfahren zur Herstellung eines Rückstandsheizöls, vorzugsweise eines Nummer 6 Heizöls, dadurch gekennzeichnet, daß in dem Heizöl eine Menge eines Additivs aufgelöst wird, das im wesentlichen aus mindestens eine Zirkoniumsalz ausgewählt aus öllöslichen Zirkoniumsalzen von (i) Alkoholen oder Phenolen mit der Formel ROH, in der R eine Hydrocarbylgruppe mit 2 bis 24 Kohlenstoffatomen ist, oder (ii) Sulfonsäuren mit der Formel RS0₃H besteht, in der R eine Alkyl-, Cycloalkyl-, Aryl-, Alkaryl- oder Aralkylgruppe ist, wobei das Sulfonatsalz ein Molekulargewicht von bis zu 2500 besitzt und die Menge des verwendeten Additivs berechnet als metallisches Zirkonium 1 bis 1000 Gew. ppm und vorzugsweise 50 bis 150 Gew. ppm beträgt.

7. Zusammensetzung nach Anspruch 6, dadurch gekennzeichnet, daß das Heizöl über 1 Gew.% Schwefel enthält.

8. Verfahren, bei dem ein Rückstandsheizöl, vorzugsweise ein Nummer 6 Heizöl verbrannt wird, dadurch gekennzeichnet, daß
(a) in dem Heizöl eine Menge gemäß Anspruch 1 oder Anspruch 2 von mindestens einem Zirkoniumsalz gemäß einem der Ansprüche 1 und 3 bis 5 aufgelöst wird und
(b) die resultierende Rückstandsheizölzusammensetzung verbrannt wird.

## Revendications

1. Composition d'huile combustible résiduelle, caractérisée par un combustible résiduel, de préférence un fuel oil no 6, contenant une certaine quantité d'un additif constitué essentiellement d'au moins un sel de zirconium choisi parmi les sels de zirconium solubles dans l'huile, (i) d'alcools ou de phénols ayant la formule ROH, dans laquelle R est un groupe hydrocarbyle de 2 à 24 atomes de carbone, ou (ii) d'acides sulfoniques ayant la formule RS0₃H, dans laquelle R est un groupe alkyle, cycloalkyle, aryle, alkaryle ou aralkyle, le poids moléculaire du sulfonate allant jusqu'à 2500 et la quantité d'additif allant de 1 à 1000 parties par million en poids, calculée en zirconium métallique.

2. Composition d'huile combustible résiduelle selon la revendication 1, caractérisé en ce que le sel ou les sels de zirconium est ou sont présent(s) en quantité totale de 50 à 150 ppm en poids, calculée en zirconium métallique.

3. Composition selon la revendication 1 ou 2, dans laquelle le groupe R de l'alcool est un groupe aliphatique saturé ou insaturé ayant 2 à 8 atomes de carbone.

4. Composition selon la revendication 1 ou 2, dans laquelle le groupe R de l'acide sulfonique est un groupe alkaryle et le sel a un poids moléculaire de 200 à 700.

5. Composition d'huile combustible résiduelle selon la revendication 1 ou 2, caractérisé en ce que le sel ou les sels de zirconium et ou sont choisi(s) parmi le propoxyde de zirconium, le dodécylbenzènesulfonate de zirconium ou les mélanges de ceux-ci.

6. Procédé de préparation d'une huile combustible résiduelle, de préférence un fuel-oil n° 6, caractérisé par la dissolution dans cette huile combustible d'une certaine quantité d'un additif constitué essentiellement d'au moins un sel de zirconium choisi parmi les sels de zirconium soluble dans l'huile (i) d'alcools ou de phénols ayant la formule ROH, dans laquelle R est un groupe hydrocarbyle de 2 à 24 atomes de carbone, ou (ii) d'acides sulfoniques ayant la formule RS0₃H, dans laquelle R est un groupe alkyle, cycloalkyle, aryle, alkaryle ou aralkyle, le poids moléculaire du sulfonate allant jusqu'à parties 2500, la quantité d'additif employé étant de 1 à 1000 parties par million, de préférence de 50 à 150 parties par million, en poids, calculée en zirconium métallique.

7. Composition selon la revendication 6, dans laquelle l'huile combustible contient plus de 1% en poids de soufre.

8. Procédé dans lequel on brûle une huile résiduelle, de préférence un fuel-oil, n° 6, caractérisé en ce que
(a) on dissout dans l'huile combustible une quantité définie dans la revendication 1 ou 2, d'au moins un sel de zirconium défini dans l'une quelconque des revendications 1 et 3 à 5, et
(b) on brûle la composition d'huile combustible résiduelle obtenue.
